

## UNITED STATES PATENT OFFICE

DONALD W. RANDOLPH AND JAY T. FORD, OF FLINT, MICHIGAN, ASSIGNORS TO A C SPARK PLUG COMPANY, OF FLINT, MICHIGAN, A COMPANY OF MICHIGAN

## DIAPHRAGM FOR FUEL PUMPS AND METHOD OF MAKING SAME

No Drawing.

Application filed December 18, 1929. Serial No. 415,116.

This invention relates to diaphragms such as are used in pumps for feeding gasoline and other liquid fuels to automobile engines and the like. It also relates particularly to methods of manufacture of such diaphragms.

In the manufacture of fuel pump diaphragms particular methods of coating and particular oil compositions are used in treating fabric materials in order to obtain the desirable physical and chemical properties. The cloth fabric must be strong enough to withstand repeated flexings and must be coated in such a manner as to be impervious to air as well as gasoline, or other liquid fuels. The coating must also be practically insoluble in liquid fuels. The coating as well as the fabric base must resist the action of repeated flexing and also must have a minimum change in flexibility with changes in operating temperatures. In particular the coated fabric must not become greatly stiffened and thus lose flexibility upon prolonged exposure to temperatures 20° below zero Fahrenheit or lower.

All of the above qualities are especially essential in diaphragms for fuel pumps used on automobile engines if the pump is to give the owner of the car uninterrupted carefree service over periods of years and in all kinds of climates.

In order to obtain these desirable physical and chemical properties it is essential, first, that a suitable textile material be employed in the diaphragms. While there is, of course, more or less latitude in the weave of the fabric and the material of which it is composed, we have found that the most suitable textile material upon which to apply the coating is a mercerized cotton fabric closely woven from two-ply yarn so as to have at least 80 threads per inch in each direction, thus forming what is known as a square woven cloth. Such fabric, properly woven, has a tensile strength of at least 80 pounds per inch width.

In order that the cloth may absorb a sufficient amount of the coating, it is essential that it be relatively free from starch. We have found it desirable to keep the starch content of the uncoated cloth under 1%.

The cloth must likewise be free from traces

of acid, which tends to weaken the fabric by slow attack, and the moisture content of the cloth must not be more than about 1%.

The fabric is obtained in large rolls and the next step consists in the coating of the cloth to render it impervious to gasoline, benzol, and the like, without rendering it too stiff for efficient use. In coating the cloth it is preferably fed through rollers into a tank containing the material for the first or base coat, is then passed through a drying oven; two coats are then applied to each side of the cloth. Drying is carried out between each successive coatings. Our invention has as one of its special objects the control of the drying operations to insure a uniform product, which will be neither too stiff not too soft, and the details of this system of control will now be described.

The first, or base coat consists of drying oils preferably applied with a suitable non-drying and non-volatile thinner. We have used with success mixtures of boiled tung oil with boiled linseed oil or boiled rubber seed oil. Such raw or partially oxidized oils which dry to a characteristic tough film are themselves soluble in gasoline and other solvents in the raw state. The film produced by drying of the oils, however, is not soluble in ordinary solvents and the extent of solubility decreases with the extent of the drying operation.

"Drying" in this discussion, is used to describe the chemical change by which a solid film is produced from an oil which is originally liquid. This is a chemical change, and is partly oxidation, partly polymerization, and perhaps other chemical changes are involved.

The raw oils, after being mixed together, are preferably partially dried by heating to a temperature of 200° F. At the same time a stream of air is passed through the oil, until the iodine number of the oil is reduced to 150 to 160 (Wijs' method). This method is described in Technical Methods of Analysis, R. C. Griffin, 1st edition, p. 241.

The mixture of oils we have found most advantageous for coating is composed of equal parts by volume of linseed oil and tung

oils partially dried as described above. The specific gravity of the mixture is 0.938 to 0.943. In applying the first coat there is added to the oil mixture 15% to 25% of one of the following classes of thinners: either

(A) A raw vegetable oil (drying oil) such as linseed, tung, perilla or rubber seed oil, or

(B) A thinner, of any suitable composition, which, for the most part, does not

10 evaporate during the drying operation. An example of such a thinner is "oleum spirits," a product of the Standard Oil Company which has an initial boiling point of 147° F., a 10% point of 309° F., and a 90% point of 15 392° F.

20 The purpose of a thinner of either class "A" or class "B" is to increase the flexibility of the coating at low temperatures, the drying operation preferably not being carried to a point where the thinner of class "A" is appreciably dried or any considerable part of the thinner of class "B" is removed by evaporation.

25 The first coat is applied as previously stated, by running the strip material through a bath containing the oils until a square yard of the cloth, absorbs approximately 2.7 ounces of the oils. The cloth is then passed through a drying oven for a sufficient length 30 of time, and with the oven maintained at a sufficient temperature so that it is dried only to the point where it ceases to be sticky.

35 It is very important that the drying be carried just far enough to produce a relatively insoluble oil film and not so far as to make the cloth so stiff at low temperatures as to interfere with the operation of the pump. We have succeeded in achieving accurate control by specifying the amount of iodine 40 that will be absorbed by one hundred grams of the oil coating, since the iodine adsorption is a measure of the state of dryness of the coating. The iodine number for the cloth thus coated is kept between 5 and 15 grams 45 per 100 grams of coating, by controlling the drying time and temperature in any suitable manner. In actual practice we have employed, with the specific cloth and composition described which is applied in three coats, 50 drying oven temperatures around 150° F., and have continued the drying treatment for 8 to 10 hours. Obviously if the temperature is increased, the time may be shortened and vice versa. But for best results the temperature should in no case exceed 160° F., particularly in drying the first coat where a non-drying thinner is used.

55 It will be found that a coating applied as described will thoroughly impregnate the fibers of the cloth and that the oil completely closes the pores of the fabric, making it air-tight.

60 The second and third coats are each applied to both sides of the fabric simultaneously as 65 by running the fabric over a roller or rollers

which are immersed in the oils. It has been found by experience that the second and third coats should be made without thinner as the solubility of the surface coating is less when the thinner is left out, and the flexibility of 70 the finished cloth is not decreased.

By the second coating the oil content of the material is increased until a square yard of the original cloth has absorbed additional oil to the amount of 1.5 ounces. The drying 75 after the second coat is accomplished in the same manner as after the first and is carried to the point where 15 to 20 grams of iodine are absorbed per hundred grams of coating. In the specific example given, the second drying 80 may be carried on at approximately 150° F. for a period of 8 to 10 hours.

85 The third coat is of the same composition and is applied in the same manner as the second, and is such as to bring the weight of the coated cloth to at least 8.8 ounces per square yard. In other words, a square yard of the original cloth has now absorbed a total of 5 ounces of oil. The drying of the third 90 coat is carried to the point where the iodine number of the finished coating is 6 to 15 grams of iodine per 100 grams of coating. The drying may be accomplished by exposing 95 the cloth to oven temperatures around 150° F. for a period of 8 to 10 hours.

100 We have found by exhaustive tests that with an iodine number below 6, diaphragms for commercial fuel pumps are so stiff as to require so many strokes to feed a given volume of fuel that the engine's supply is seriously interfered with. The result is poor engine operation. We have likewise found by tests that with an iodine value above 15 the solubility of the coating in gasoline becomes excessive and it becomes so soft as to rub off 105 in handling, particularly when exposed to gasoline, kerosene or the like.

110 Diaphragms are now cut from the finished fabric, each diaphragm comprising a number of layers of the coated cloth. Before assembling the diaphragms in the pump we have found it necessary to further soften the cloth coating by immersion in kerosene for a period of about twenty minutes. The action of the kerosene is such as to soften the coating and 115 reduce its tendency to stiffen at low operating temperatures.

120 We want to particularly emphasize the importance of accurate control of drying as set forth in this application. Without this the coated fabric will be found to vary in physical properties to such extremes that the coating will rub off because of its softness or it will become so stiff at lower temperatures that it will not be flexible enough to function 125 properly. We have found it to be impossible to obtain a satisfactory commercial product without such control of the drying process.

130 If desired more or less than the three coats herein specified may be used although we

have found the specific cloth treatment herein described to be best.

In the specification we have referred to both linseed and rubber seed oils as being usable interchangeably in conjunction with tung oil to produce a satisfactory coating. In the absence of an established class name, we have used the phrase 'oil selected from a group consisting of "linseed oil and rubber seed oil"' as descriptive of either of the oils alone or a combination of the two.

We claim:

1. A diaphragm for fuel pumps comprising cloth impregnated with a partially dried mixture of tung and rubber seed oils.

2. A diaphragm for fuel pumps comprising cloth impregnated with a partially dried mixture of tung oil and oil selected from a group consisting of linseed oil and rubber seed oil in substantially the proportions of 1 to 1 by volume.

3. A diaphragm for fuel pumps comprising cloth impregnated with a coating of a partially dried mixture of tung oil and oil selected from a group consisting of linseed oil and rubber seed oil in substantially the proportions of 1 to 1, applied with a thinner, to render it impervious to air and insoluble in liquid hydrocarbon fuels, said cloth having on its surfaces a dried layer of the said oils, applied without a thinner.

4. A diaphragm for fuel pumps comprising cloth impregnated with a coating of a partially dried mixture of tung oil and oil selected from a group consisting of linseed oil and rubber seed oil in substantially the proportions of 1 to 1, applied with a thinner, to render it impervious to air and insoluble in liquid hydrocarbon fuels, said cloth having on its surfaces dried layers of the said oils in the same proportions and applied without a thinner.

5. A diaphragm for fuel pumps comprising fabric provided with a partially dried coating of drying oils, the coating having an iodine number of from 6 to 15.

6. A diaphragm for fuel pumps made of fabric substantially free of starch, acid and moisture, and provided with a partially dried coating of drying oils having an iodine number of from 6 to 15.

7. A diaphragm for fuel pumps made of fabric substantially free of starch, acid and moisture, and provided with a partially dried coating of a mixture of tung oil and oil selected from a group consisting of linseed oil and rubber seed oil, the coating having an iodine number of from 6 to 15.

8. A diaphragm for fuel pumps made of fabric substantially free of starch, acid and moisture and impregnated and coated with a partially dried coating of a mixture of tung oil and oil selected from a group consisting of linseed oil and rubber seed oil.

9. The method of making a fuel pump dia-

phragm adapted to resist hydrocarbon fuels and to remain flexible throughout a wide temperature range which consists in thoroughly impregnating fabric with a mixture of tung oil and oil selected from a group consisting of linseed oil and rubber seed oil, and drying the cloth until the coating shows an iodine number of from 6 to 15.

10. The method of making a fuel pump dia-phragm adapted to resist the action of hydro-carbon fuels and to remain flexible throughout a wide temperature range consists in im-pregnating fabric with a mixture of tung oil, oil selected from a group consisting of lin-seed oil and rubber seed oil, and a non-vola-tile thinner, drying the treated cloth, and coating it with a mixture of the said oils ap-plied without the thinner, and so drying the coated cloth that the coating shows an iodine number of from 6 to 15.

11. The method of making a fuel pump dia-phragm adapted to resist hydrocarbon fuels and to remain flexible throughout a wide tem-perature range which consists in thoroughly im-pregnating fabric with a mixture of tung oil and oil selected from a group consisting of linseed oil and rubber seed oil in substantially the proportions of 1 to 1 by volume, applied with a suitable thinner, partially drying the im-pregnated fabric, coating the im-pregnated fabric with a mixture of the oils in the same proportions and drying the coated and im-pregnated fabric until the coating has an iodine value of 6 to 15.

12. The method of making a fuel pump dia-phragm adapted to resist the action of hydro-carbon fuels and to remain flexible throughout a wide temperature range which consists in im-pregnating fabric with a mixture of tung oil, oil selected from a group consisting of linseed oil and rubber seed oil, and a thinner, drying the fabric until the coating shows an iodine number of 20 to 30, applying a mixture of the said oils to opposite sides of the fabric and drying the coated fabric until the coat-ing shows an iodine number of from 6 to 15.

13. The method of making a fuel pump dia-phragm adapted to resist the action of hydro-carbon fuels and to remain flexible throughout a wide temperature range which consists in im-pregnating fabric with a mixture of tung oil, oil selected from a group consisting of linseed oil and rubber seed oil, and a thinner, drying the fabric until the coating shows an iodine number of 20 to 30, applying a mix-ture of the said oils to both sides of the treated fabric, and drying the coating until it shows an iodine number of from 15 to 20, applying a third coating of the mixture of the said oils to both sides of the treated fabric and drying the fabric until the coating shows an iodine number of from 6 to 15.

14. The method of making a fuel pump dia-phragm adapted to resist hydrocarbon fuels and to remain flexible throughout a wide tem-

perature range which consists in thoroughly impregnating and coating fabric with a partially dried mixture of drying oils, and softening the coating by immersing the diaphragm in a suitable liquid for a short period prior to assembly, whereby the liquid together with the fuel in contact with the diaphragm assist in maintaining the flexibility of the diaphragm during use.

10 15. A coated fabric resistant to the action of hydrocarbon fuels and the like consisting of cloth impregnated with a partially dried mixture of tung and rubber seed oils.

In testimony whereof we affix our signatures.

15 JAY T. FORD.  
DONALD W. RANDOLPH.

20

25

30

35

40

45

50

55

60

65